

## UNITED STATES PATENT OFFICE

2,218,618

## LUBRICANT

John G. McNab, Roselle, and Walter T. Watkins,  
 Jr., Elizabeth, N. J., assignors to Standard Oil  
 Development Company, a corporation of Dela-  
 ware

No Drawing. Application February 25, 1939,  
 Serial No. 258,456

9 Claims. (Cl. 252—32)

The present invention relates to lubricants and more particularly to lubricating oils containing polyvalent metal soaps which are useful for many purposes, but especially for the lubrication of 5 Diesel engines. The invention will be fully understood from the following description.

It has been found desirable in many cases to add relatively small amounts of polyvalent metal salts of organic acids to lubricating oils, but difficulty has been met in obtaining suitable acids for the purpose. The common saturated acids of commerce, such as stearic, margaric, and palmitic, form heavy metal soaps which are not very soluble, especially in paraffinic oils and for this 15 reason they cannot be used. Naphthenic acids have not proven wholly satisfactory.

It has been found that suitable acids can be obtained quite cheaply as a by-product of the oxidation of hydrocarbons, especially waxy hydrocarbons. Materials such as paraffin wax, petrodatum, especially deoiled petrodatum, and highly purified hydrocarbon oils may be oxidized with air or oxygen at relatively low temperatures, that is from about 100 to 150° C., especially with the 20 use of catalysts such as barium or magnesium soaps, manganese salts and the like, so as to produce large yields of readily distillable acids of the molecular weight range, comparable to the acids used in soap manufacture. In addition to 25 this main product, there is a minor amount of an acidic product of uncertain constitution, probably polymerized to a considerable extent, which is substantially undistillable even under vacuum or with steam. This material contains a large 30 percentage of free acids of high molecular weight which can be used for the present purposes, as well as combined acids which may also be used if desired.

The undistillable product referred to above 35 may be separated from the lower acids and the unoxidized hydrocarbon in a number of different ways, but it has been found preferable to saponify the crude product of oxidation with aqueous caustic under pressure. The mixture obtained 40 is fluid and its tendency to emulsify can be counteracted by the addition of alcohol. The aqueous fluid is then preferably extracted with kerosene and naphtha so as to remove the unoxidized hydrocarbon and the alcohol may be distilled and 45 recovered. The organic acids are regenerated by reacidification and form a layer which is decanted from the aqueous solution.

This organic layer may be purified further and it is then distilled under vacuum or with steam. The distillate is largely composed of acids of 12 to

18 or 20 carbon atoms and distillation is continued until substantially all of the material that can be vaporized without decomposition is removed, so as to leave as a residue the acidic substantially non-distillable by-product which is the 5 subject of the present invention. The chemical nature of this residue is not fully understood, but a partial analysis shows the following:

|                          | Percent | 10 |
|--------------------------|---------|----|
| Free acid.....           | about   | 30 |
| Esters and lactones..... |         | 65 |
| Unsaponifiable.....      |         | 5  |

The total residue as obtained above has a neutralization value of 46 mg. KOH/gr., and a saponification value, which is obtained by refluxing with KOH, of 175 mg. KOH/gr. When the refluxing is conducted under pressure, a higher value of 200 mg. KOH/gr. for the saponification number is obtained. From the above, it will be 15 seen that this material is quite different from ordinary fats and waxes. It is substantially free of aldehydes and aldehyde-like bodies and due to polymerization is of considerably higher molecular weight than the wax or other hydrocarbon from which it is produced, and likewise higher than the molecular weight of other acids readily available commercially.

In producing the polyvalent metal soaps, the free acid content of the undistillable oxidation 30 by-product may be used alone. The free acids may be roughly separated from non-acidic bodies and combined acids by solution in alcoholic caustic soda, and after separation of these soda soaps or salts, their reaction may be effected with 35 water soluble salts of the particular polyvalent metal or metals which are desired. If desired, the total oxidation product may be used and in this case it may be desirable to produce the soda salts by saponification under pressure so as to convert 40 at least a portion of the combined acids into soda soaps as well as the free acids. These soaps may then be purified and converted into heavy metal soaps as disclosed above.

If the total undistillable residue is employed 45 in producing soda soaps, the mixture then contains a considerable amount of unsaponifiable materials and, indeed, even if the roughly purified acids are used there is a certain amount of unsaponifiable material in the heavy metal soap 50 mixture, and it has been found desirable to remove at least the larger portion of such impurities. This can be accomplished in several different ways, but the best method is by extraction of the heavy metal soap with low molecular

weight oxygen-containing solvents such as ethyl or methyl alcohol, propyl or butyl alcohols or, if desired, ketones of the same general molecular weights may be employed. In this manner, 5 the nonsaponaceous materials are removed from the heavy metal soaps or, at least, their proportion is so reduced as to make little or no detriment.

Various polyvalent metal soaps can be made 10 by the above described methods, but the ones which are of the most importance for the present invention are the alkaline earth metal soaps, principally those of calcium and magnesium and also the soaps of aluminum, lead, zinc, and chromium, as well as the soaps of the 8th Group metals, particularly nickel and cobalt. Among the various advantages obtained by the use of these soaps of the high molecular weight acids is the greatly increased solubility in various oils, 15 not only of the naphthenic type but likewise of the paraffinic.

Soaps of the different polyvalent metals have somewhat different properties, but all may be added to oils in proportions ranging from about 20 .10 to 3% or even 5% for specific purposes. These soaps dissolve readily and do not tend to separate out or gel on standing as is the case with similar soaps of the commercial fatty acids of the type of stearic acid.

30 The soaps of the acids as prepared above are also found to have a marked solubilizing effect on soaps of the saturated acids, such as stearic, so that it is quite advantageous in many instances to use mixtures of soaps of stearic or 35 margaric or other acids of the same class together with those of the higher molecular weight, such as described above, without danger of separation on standing. The proportion of the heavy molecular weight soaps necessary to effect the solubilizing depends on various factors, 40 principally on the particular metal soaps employed, the oil in which they are used and also the amount or proportion of the total soap to be put into the oil. In general, equal amounts of 45 the higher and the lower molecular weight soaps, such as those of stearic acid, will be sufficient to insure solubility, although less may be employed in many instances and a greater proportion of the heavier molecular weight soap is 50 found to be unobjectionable. In any particular instance, the most desirable amount can be readily found by experiment.

The soaps disclosed above are especially useful in oils for the lubrication of Diesel engines 55 and are found to reduce wear and generally to improve performance, but especially to maintain a clean engine condition particularly in the pis-

aluminum soaps or of calcium and nickel, or even mixtures of the three or more soaps.

These soaps may comprise the only addition agents which are employed, or they also may be used with other materials. It is found, for example, that small amounts of free stearic acid are quite desirable in the oils for certain purposes; also that heavier compounds, especially 5 corrosive sulfur compounds, are used together with the lead and/or zinc soaps for extreme pressure purposes. The soaps may be employed along with thickening agents, pour point depressants, sludge dispersing agents or various other materials which have some special use for 10 particular service.

#### EXAMPLE 1

Calcium soaps were prepared from stearic acid and distilled acids obtained from the oxidation of sweater oil (oil sweated from wax). Neither of these calcium soaps could be dissolved in oil. A calcium soap was then prepared from the substantially undistillable bottoms obtained in the distillation of oxidized wax acids and it was found readily soluble in mineral oils. The aluminum soap of the bottoms was then prepared and found very freely oil-soluble. Aluminum stearate, although initially oil-soluble, causes gel formation on cooling.

#### EXAMPLE 2

Calcium soaps were subsequently prepared from: (1) A 50-50 mixture of stearic acid and substantially non-distillable oxidized acids obtained by wax distillation, (2) A 50-50 mixture of distilled sweater oil acids and the non-distillable acids. The calcium soap mixtures were readily oil-soluble in both instances, giving bright, clear blends stable on storage for several months. An aluminum soap was subsequently prepared from a mixture containing 90% stearic acid and 10% non-distillable acids. This soap also proved readily oil-soluble. These data demonstrate the solubilizing effect of the soaps prepared from non-distillable acids. The three soaps mentioned above were blended in separate 35 samples of naphthenic oils and a blend of each soap tested in a CFR engine test (375° F. jacket 40 temperature, 14-hour test). All soaps produced an improvement in engine performance as will be seen from the data below. After each test 45 the engine was taken down and the pistons carefully examined and rated on the basis of their condition and cleanliness. From the rating of the separate parts of the piston assemblies, an overall rating was recorded. It should be noted 50 that these ratings are demerits and the smaller numbers indicate superior performance.

#### CFR Engine tests: 375° F. jacket temperature

| 60 | Samples                                                                          | Overall demerit | Rings stuck | Ring slits | Ring grooves | Carbon under-side | Varnish skirt | 60 |
|----|----------------------------------------------------------------------------------|-----------------|-------------|------------|--------------|-------------------|---------------|----|
| 65 | Essolube 30 (Ref.)                                                               | 4.36            | 3           | 8.33       | 6.5          | 4                 | 5             |    |
|    | Oil+1.0% calcium soap of 50/50 (distilled sweater oil acids+undistillable acids) | 1.39            | 0           | 1.00       | 4.5          | 1.5               | 0.5           | 65 |
|    | Oil+1.0% calcium soap 50/50 (stearic acid+undistillable acids)                   | 2.22            | 0           | 1.33       | 6.0          | 3                 | 2             |    |
|    | Oil+1.0% aluminum soap (90% stearic acid+10% undistillable acids)                | 1.62            | 0           | 1.00       | 5.5          | 3                 | 4             |    |

70 ton assemblies, rings, slits, grooves, and the like, and to reduce gummy or varnish-like deposits. For use in Diesel engines, the single soaps, particularly those of calcium, aluminum, chromium, nickel, and cobalt, are quite satisfactory but even better results may be obtained by using mixed 75 soaps, for example, mixtures of calcium and

#### EXAMPLE 3

70 A 1% blend of the calcium soap prepared from distilled sweater oil acids and undistillable acids in a naphthenic base stock was tested for a long period (almost 500 hours) in a Caterpillar Diesel engine. In this test marked reduction in cylinder 75

der wear and improvement in overall engine performance were obtained as evident from the attached data.

carbon oxidation product, reacidification and distillation of the volatile acids so as to leave a substantially non-distillable acid as a residue.

*Caterpillar single cylinder engine tests*

| Eng.<br>No. | Run<br>No. | Oil                                                                                   | Hours | Overall<br>piston<br>demerit | Demerits              |         |        |             |                       |                        | Liner<br>wear per<br>1000 hrs. | 5     |    |  |
|-------------|------------|---------------------------------------------------------------------------------------|-------|------------------------------|-----------------------|---------|--------|-------------|-----------------------|------------------------|--------------------------------|-------|----|--|
|             |            |                                                                                       |       |                              | Ring zone cleanliness |         |        | Car-<br>bon | Skirt<br>and<br>liner | Varnish<br>on<br>skirt | Oil<br>filter                  |       |    |  |
|             |            |                                                                                       |       |                              | Slits                 | Grooves | SGLS * |             |                       |                        |                                |       |    |  |
| 10          | C1         | Naphthenic base stock                                                                 | 100   | 2.13                         | 0                     | 2.8     | 1.69   | 4.8         | 4.00                  | 4                      | 0                              | .0063 | 10 |  |
|             |            | Naphthenic base stock<br>+1.0% calcium soap 50/50                                     | 126   | 1.22                         | 0                     | 2.6     | 1.45   | 4.7         | 0.83                  | 1.5                    | 1                              | ----- |    |  |
| 15          | C1         | +1.0% calcium soap 50/50<br>(distilled sweater oil acids<br>and undistillable acids). | 278   | 1.54                         | 0.5                   | 3.4     | 1.94   | 5           | 1.5                   | 1                      | 2                              | .0039 | 15 |  |
|             |            |                                                                                       | 491   | 2.10                         | 2                     | 4.3     | 2.96   | 5.9         | 2.00                  | 2                      | 2                              | .0016 |    |  |

\*Cleanliness of ring slits, grooves, lands, and sides.

The present invention is not to be limited by any specific examples which have been presented herein solely for the purpose of illustration, but only by the following claims in which it is desired to claim all novelty inherent in the invention.

We claim:

1. An improved lubricant comprising a mineral lubricating oil and a polyvalent metal soap of substantially non-distillable organic acids obtained as a by-product of the oxidation of petroleum hydrocarbons.
2. An improved lubricant comprising a mineral lubricating oil and a polyvalent metal soap of substantially non-distillable high molecular weight acid obtained as a by-product of wax oxidation.
3. An improved lubricant comprising a mineral lubricating oil and 1 to 5% of a polyvalent metal soap of a substantially non-distillable organic acid obtained by neutralization of a crude hydro-

4. Product according to claim 3 in which the soap is an alkaline earth metal soap.

5. Product according to claim 3 in which the soap is a calcium soap.

6. Product according to claim 3 in which the soap is a cobalt soap.

7. Product according to claim 3 in which the soap is a soap of the 8th Group metals.

8. Product according to claim 3 in which the soap is a nickel soap.

9. An improved lubricant for Diesel engines consisting of a mineral lubricating oil and a small amount of a polyvalent metal soap, of the substantially non-distillable high molecular weight acids obtained as a by-product in the oxidation of waxy hydrocarbons.

JOHN G. McNAB.

WALTER T. WATKINS, JR.

35

20

25

30